

## UNITED STATES PATENT OFFICE

2,131,320

## PRINTING WITH MORDANT DYESTUFFS

Emil Gubler, Basel, Switzerland, assignor to the  
firm Durand & Huguenin S. A. Basel, Switzerland

No Drawing. Application February 2, 1937, Serial No. 123,726. In Germany February 11, 1936

7 Claims. (Cl. 8—72)

In the U. S. patent application Ser. No. 716,091 are described processes for printing with mordant dyestuffs (chrome dyestuffs) on fabrics of animal fibres, namely natural silk, and on fabrics of regenerated cellulose such as viscose artificial silk, cuprammonium artificial silk and so on, in which the printing pastes used contain the mordant dyestuff, gum arabic thickening and a chromium mordant, having Cr in the cation in the presence of a lactate group. The principal advantage of the processes is to be found in the fact that the soft feel and the lustre of the fibre, which in the absence of the lactate group, owing to coagulation of the arabic gum thickening in presence of the chromium mordant, would suffer, are retained. According to a particularly advantageous form of the processes chromium lactate is used. The processes may also be combined with advantage with the process of U. S. Patent No. 1,848,589, according to which urea is also used in the printing paste.

According to the hitherto usual procedure, after the prints thus prepared have been steamed they must be washed first with cold water and then with lukewarm water at about 40–50° C. in order that the fibres may have the desired soft feel. This procedure involves certain disadvantages. For example, if basic dyestuffs are printed on the material together with the chrome dyestuffs, the prints of the basic dyestuffs are damaged by the treatment with lukewarm water and bleed. Moreover, the apparatus necessary for the treatment is not available in all silk printing works.

The present invention relates to an improvement whereby the treatment with lukewarm water is rendered unnecessary, and a completely soft feel of the fibres is attained by simply washing the printed material with cold water after steaming. For this purpose in accordance with the invention there is added to the printing paste sodium tartrate or, in general, an alkali salt of an aliphatic oxy acid such as tartaric acid, lactic acid, glycollic acid and so on.

If, as has hitherto been preferable, chromium lactate is used in the known process the present invention may be carried into effect by adding an alkali lactate, alkali tartrate or alkali glycolate to the printing paste in addition to chromium lactate.

The following examples illustrate the invention:

The following printing pastes are prepared:

| Example                                                            | 1        | 2     | 3     | 5     |
|--------------------------------------------------------------------|----------|-------|-------|-------|
| Chromocitronine R (Schultz, Farbstofftabelle 5 7th Edn., No. 432)  | Grams 30 |       |       |       |
| Chromacetine blue S (Schultz, Farbstofftabelle 7th Edn., No. 999)  |          | 30    |       | 10    |
| Dyestuff according to Example 1 of German Specification No. 456234 |          |       | 30    |       |
| Water                                                              | 232      | 192   | 152   |       |
| Formic acid (30%)                                                  |          | 30    |       |       |
| Phenol                                                             |          |       | 30    |       |
| Furfuryl alcohol                                                   |          |       | 10    |       |
| Sodium tartrate cryst.                                             | 30       | 30    | 30    |       |
| Gum arabic thickening (1:1)                                        | 610      | 610   | 610   |       |
| Chromium lactate (14.7% Cr <sub>2</sub> O <sub>3</sub> )           | 38       | 38    | 38    | 15    |
| Urea                                                               | 60       | 60    | 100   |       |
| 25% solution of hydrosulphite NF                                   |          | 10    |       |       |
|                                                                    |          | 1,000 | 1,000 | 1,000 |

The paste is printed on natural silk or viscose artificial silk, and the material is steamed for 45 minutes, then washed with cold water and dried. There are obtained respectively yellow, blue and orange prints whilst the fibre has an unobjectionable soft feel.

In the case of Example 2 the duration of the steaming can be appreciably shortened by increasing the quantity of urea to 100 grams.

Sodium lactate or sodium glycolate can be used instead of sodium tartrate in the foregoing examples with similar effect.

The invention may also be applied in printing fabrics of other artificial silks, such as fabrics of cuprammonium artificial silk.

What I claim is:—

1. In a process of steam printing with chromium mordant dyestuffs on lustrous fibres, including natural silk and regenerated cellulose fibre, such as viscose or cuprammonium artificial silk, an improvement consisting in printing the material with a paste containing the mordant dyestuff, a gum arabic thickening, a chromium mordant having Cr in the cation in the presence of a lactate group, and an alkali salt of an aliphatic hydroxy acid, thereby obviating the formation of a harsh feel, uneven dyeing and loss of lustre on the imprinted parts.

2. In a process of steam printing with chromium mordant dyestuffs on lustrous fibres, including natural silk and regenerated cellulose

35

25

30

35

20

30

40

45

50

- fibre such as viscose or cuprammonium artificial silk, an improvement consisting in printing the material with a paste containing the mordant dyestuff, a gum arabic thickening, chromium lactate, and an alkali salt of an aliphatic hydroxy acid, thereby obviating the formation of a harsh feel, uneven dyeing and loss of lustre on the imprinted parts.
3. As a new composition of matter, a printing paste containing a mordant dyestuff, a gum arabic thickening, a chromium mordant having Cr in the cation in the presence of a lactate group and an alkali salt of an aliphatic hydroxy acid.
5. A printing paste containing a mordant dye-  
stuff, a gum arabic thickening, chromium lactate and an alkali salt of an aliphatic hydroxy acid.
5. A printing paste containing a mordant dye-  
stuff, a gum arabic thickening, chromium lactate and sodium tartrate.
6. A printing paste containing a mordant dye-  
stuff, a gum arabic thickening, chromium lactate and sodium glycollate.
7. A printing paste containing a mordant dye-  
stuff, a gum arabic thickening, chromium lactate and sodium lactate.
- 10

EMIL GUBLER.